

# United States Patent Office

2,756,151

Patented July 24, 1956

1

2,756,151

## REDUCTION OF DYE STAIN IN PROCESSED PHOTOGRAPHIC PAPERS CONTAINING DYES

Walter J. Weyerts, Rochester, N. Y., assignor to Eastman Kodak Company, Rochester, N. Y., a corporation of New Jersey

No Drawing. Application August 1, 1952,  
Serial No. 302,237

5 Claims. (Cl. 95—88)

This invention relates to the reduction of dye stain in processed photographic papers containing sensitizing dyes by the addition of aryl or alkaryl sulfonic acids or their water-soluble salts to the stop bath or the fixing bath which are employed in processing those papers.

The emulsions employed for photographic papers often contain sensitizing dyes and many of the dyes of this nature have a tendency to introduce stain into the paper upon the processing of those papers. This effect has been noted, for instance, in the case of papers for producing direct positive photographs, for example, of the type described in U. S. Patent No. 2,497,875 of George E. Falleson. Also, in cases where dyes have been used in higher than normal concentration, or in some cases of special processing, my invention finds application. Types of sensitizing dyes which, when used in photographic paper emulsions, have a tendency to stain the paper upon its processing are acid type dyes such as the merocyanines, the eosins, the oxonols and the acid azo dyes, such as Congo red and Glycine red.

One object of my invention is to provide a procedure for processing photographic paper in which staining of the paper by the sensitizing dye in the photographic emulsion used is substantially eliminated. Another object of my invention is to provide a method for processing photographic papers in which an aryl or alkaryl sulfonic acid or its soluble salt is employed in the stop bath or the fixing bath in which the paper is processed. A further object of my invention is to prevent staining of photographic paper in the machine processing of photographic paper in which the washing time is relatively short (such as less than 4 minutes). Where a relatively long time of washing is employed, such as on the order of 10 minutes, staining of the paper is negligible. Other objects of my invention will appear herein.

In the use of photographic papers, the paper is exposed, thereby producing a latent image in the emulsion thereof. The paper ordinarily is then put through a development bath to bring out the image, followed by immersion in an acid stop bath to end the development and then in a fixing bath to fix the print so obtained. It has been found that, with certain types of dyes, a short washing time, as used in machine processing, contributes to staining of the paper by those dyes, and, to prevent or minimize such staining, an aryl sulfonic acid, an alkaryl sulfonic acid or a soluble salt of one of these is added to the acid stop bath or to the fixing bath in accordance with my invention.

Some of the sulfonates which have been found to be especially useful in accordance with my invention are sodium anthraquinone-beta-sulfonate, sodium anthraquinone-alpha-sulfonate and sodium -m- terephenyl-4'-sulfonate. For instance, the use of sodium anthraquinone-beta-sulfonate in an acid stop bath in a concentration of 0.5% almost completely eliminated dye stain in processed paper, and the other sulfonates mentioned were substantially equally effective. Other compounds which exhibited a stain-reducing effect when used in the acid stop

2

bath or in the fixing bath in addition to those mentioned above were naphthalene sulfonic acids, naphthol sulfonic acids, naphthyl amine sulfonic acids, alkyl naphthalene sulfonic acids, diphenyl disulfonic acids, p-toluenesulfonic acids and salts thereof. Another material which is effective is Tamol, which is the sodium salt of naphthalene sulfonic acid condensed with formaldehyde.

These sulfonates or sulfonic acids are generally effective in concentrations within the range of 0.1-1%, but higher concentrations than the range given can be employed in stop baths or fixing baths in accordance with my invention, and in some cases the use of higher concentrations than 1% are even preferred, such as where dye staining is especially pronounced.

The processing of a photographic paper, such as of the type described in Patent No. 2,497,875 of Falleson, may be carried out by developing that emulsion layer, after its exposure, in a developer of the type disclosed and claimed in application Serial No. 218,071 of Russell and Haist, now U. S. Patent 2,625,475, such as for approximately 1½ minutes. After this development the paper is placed in an acid stop bath, such as a 3% aqueous solution of citric acid or acetic acid, such as for approximately ½ minute. The paper is then placed in a fixing bath, such as for approximately 2 minutes, which bath may have a formula as follows:

### FIXING BATH

|    | Grains                           |
|----|----------------------------------|
| 30 | Sodium thiosulfate (hypo) -----  |
|    | 300.0                            |
|    | Sodium bisulfite -----           |
|    | 7.5                              |
|    | Sodium sulfite (desiccated)----- |
|    | 7.5                              |
|    | Sodium citrate -----             |
|    | 2.0                              |
|    | Ammonium sulfate -----           |
|    | 30.0                             |
| 35 | Water to make 1 liter            |

The paper is then washed, such as in running water, for approximately 2½ minutes and dried. Without the benefit of my invention (unless long-time washing is used), the final prints ordinarily exhibit an objectionable amount of dye stain. The following examples of stop or fixing baths which can be employed in accordance with my invention to prevent the dye staining in the processing described are illustrative:

#### Example 1

45 A photographic paper having a silver bromoiodide emulsion thereon, which emulsion contained a staining sensitizing dye of the acid type, was processed as described above, but a stop bath consisting of an aqueous solution containing 3% of citric acid and 0.5% of sodium anthraquinone-beta-sulfonate was employed. The resulting paper, after fixing, washing and drying, was found to have little, if any, stain thereon.

#### Example 2

55 A photographic paper was processed as described above, however, a stop bath consisting of an aqueous solution of citric acid, 3% concentration and 0.5% of sodium -m- diphenylbenzene sulfonate was employed. After fixing, washing and drying, a paper was obtained substantially free from dye stain.

#### Example 3

65 A photographic paper, after exposure, was processed as described above using as the stop bath therein an aqueous solution containing 3% of citric acid and 1% of dibutyl phenyl phenol sodium disulfonate. The paper obtained had little or no noticeable dye stain therein.

#### Example 4

An exposed photographic paper was processed as de-

scribed above, but a fixing bath having the following formula was employed:

## FIXING BATH

|                                         | Grams |
|-----------------------------------------|-------|
| Sodium thiosulfate (hypo)               | 300.0 |
| Sodium bisulfite                        | 7.5   |
| Sodium sulfite (desiccated)             | 7.5   |
| Sodium citrate                          | 2.0   |
| Ammonium sulfate                        | 30.0  |
| Monobutyl biphenyl sodium monosulfonate | 2.0   |
| Water to make 1.0 liter                 |       |

After fixing, the paper was then washed and dried, and was found to be free of any appreciable stain from the sensitizing dye employed in the photographic emulsion.

I claim:

1. In the processing of silver halide sensitized papers containing sensitizing dyes in which the paper after exposure is developed, fixed and washed, the method of reducing dye stain in the processed, washed and dried paper which comprises treating the paper in the processing operation between the developing and final washing steps with a fixing bath containing in solution therein a compound selected from the aryl and alkaryl sulfonic acids and their water soluble salts.

2. In the processing of silver halide sensitized papers containing sensitizing dyes in which the paper after exposure is developed, fixed and washed, the method of reducing dye stain in the processed, washed and dried paper which comprises treating the paper in the processing operation between the developing and final washing steps with a fixing bath containing sodium anthraquinone- $\beta$ -sulfonate.

3. In the processing of silver halide sensitized papers

containing sensitizing dyes in which the paper after exposure is developed, fixed and washed, the method of reducing dye stain in the processed, washed and dried paper which comprises treating the paper in the processing operation between the developing and final washing steps with a fixing bath containing sodium m-terephenyl-4'-sulfonate.

4. In the processing of silver halide sensitized papers containing sensitizing dyes in which the paper after exposure is developed, fixed and washed, the method of reducing dye stain in the processed, washed and dried paper which comprises treating the paper in the processing operation between the developing and final washing steps with a fixing bath containing sodium m-diphenyl benzene sulfonate.

5. In the processing of silver halide sensitized papers containing sensitizing dyes in which the paper after exposure is developed, fixed and washed, the method of reducing dye stain in the processed, washed and dried paper which comprises treating the paper in the processing operation between the developing and final washing steps with a fixing bath containing monobutyl diphenyl sodium sulfonate.

## References Cited in the file of this patent

## UNITED STATES PATENTS

|           |                |                |
|-----------|----------------|----------------|
| 2,322,084 | Young et al.   | June 15, 1943  |
| 2,367,516 | Muehler et al. | Jan. 16, 1945  |
| 2,428,208 | Edgerton       | Sept. 30, 1947 |
| 2,440,954 | Jennings       | May 4, 1948    |
| 2,453,347 | Russell        | Nov. 9, 1948   |
| 2,578,075 | Kienast        | Dec. 11, 1951  |
| 2,615,807 | Umberger       | Oct. 28, 1952  |